

No. 656,077.

Patented Aug. 14, 1900.

G. ALEFELD.

MANUFACTURE OF INCANDESCENT MATERIALS FOR ELECTRIC LIGHTING.

(Application filed June 15, 1899.)

(No Model.)

Fig. 1.



Fig. 2.

Fig. 3.



Fig. 4.



Witnesses:

W. M. Long.  
Ethos Loftus

Fig. 5.



Inventor:

George Alefeld,  
by W. L. Smith,  
Associate Attorney.

# UNITED STATES PATENT OFFICE.

GEORG ALEFELD, OF DARMSTADT, GERMANY, ASSIGNOR TO LUDWIG  
WILHELM GANS, OF FRANKFORT-ON-THE-MAIN, GERMANY.

## MANUFACTURE OF INCANDESCENT MATERIALS FOR ELECTRIC LIGHTING.

SPECIFICATION forming part of Letters Patent No. 656,077, dated August 14, 1900.

Application filed June 15, 1899. Serial No. 720,718. (No model.)

*To all whom it may concern:*

Be it known that I, GEORG ALEFELD, a citizen of Germany, and a resident of Darmstadt, in the Empire of Germany, have invented a new and useful Improvement in the Manufacture of Incandescent Materials for Electric Lighting, of which the following is a specification.

It has been long known that certain refractory bodies—such as, for example, porcelain, magnesia, lime, zirconia, &c.—emit a brilliant light when heated to a sufficiently-high temperature. Since the heating effect of the electric current has been known numerous attempts have been made to take advantage of this property and render these bodies available for practical illumination. The production and introduction as a practical illuminant by Auer von Welsbach of bodies which become incandescent when heated by a gas-flame gave a new impulse to efforts in this direction, the more particularly since through his publications the number of known "luminous earths" has been considerably increased. The first attempt of this kind which attracted special attention was the so-called "Jablochkoff" lamp; but its practical defects were found to so outweigh its merit that it soon disappeared from the field. Walther Nernst has lately again taken up this idea and has constructed incandescents called, after his name, the "Nernst" lamp. With both the Jablochkoff and Nernst lamps the principal difficulty consists in the initial heating of the incandescent body to a sufficiently-high temperature, an initial step rendered necessary by the fact that all these luminous earths conduct the electric current very poorly at normal temperatures and only become good conductors after their temperature has been considerably raised. It is therefore necessary first to heat the to-be-incandescent body by a gas-burner or some other extraneous source of heat or means of heating before it will pass the electric current and through its action become incandescent. Jablochkoff, for example, held his incandescent body between a pair of tongs, the arms of which were connected with the conducting-wires of an electric current, connecting the said arms with the incandescent by a thin

filament of a carbon-containing material, by which the current first passed. This heated the filament, which in turn heated the to-be-incandescent body until it became itself a conductor and actually incandescent. The carbon filament was, however, destroyed in this operation and had to be replaced by a new filament every time the lamp was used. Nernst seeks to accomplish this result by leading the electric current through a coil of thin platinum wire, thus heating the coil, which in turn heats the to-be-incandescent body sufficiently to enable it to pass the current when it becomes incandescent and at the same time the heating-coil is automatically cut out of the circuit.

The object of my invention is to accomplish the same ultimate result in a much more simple, effective, and durable way and at the same time dispense with all sources and means of extraneous initial heating not so united to the incandescent body as to form practically an integral part thereof. Moreover, my initial heating device is not only capable of prolonged repeated use without impairment, but it also dispenses with any form of cutting-out device, since it remains constantly in circuit while my lamp is in operation.

In the drawings forming part of this specification, Figure 1 represents a perspective view and an axial section of an improved incandescent in the form of a hollow cylinder. Figs. 2 and 3 are like views and sections of improved incandescents in the form of curved tubes. Fig. 4 represents a magnified cross-section through either of said hollow and tubular incandescents, and Fig. 5 represents a perspective view and cross-section of another form.

Like letters refer to like parts in all the figures.

My improved incandescent is composed of a suitable body *a*, composed of one or more of those oxides of the earthy metals which become luminous at elevated temperatures and a film-like partial coating *b* of one or more of the highly-infusible metals of the platinum group to constitute a practically-indestructible preliminary conductor, and it is in practice used in connection with a suitable elec-

tric contact which may answer for both the body *a* and the conductor *b* with or without an inclosing bulb, as hereinafter more particularly described.

5 The preliminary conductor *b* is of necessity greatly exaggerated as to thickness in the drawings. To produce this preliminary conductor *b*, forming my initial heating device, I use the so-called "ceramic lustrous preparations of the noble metals," which, as well as the art of burning them in, are well known in the art of china and glass decoration and are regularly made and sold for that purpose. They are organic compounds of the 10 noble metals—gold, silver, and the metals of the platinum group, (resin-acid compounds or sulfureted resin-acid compounds, the products of the decomposition of metallic chlorids by heating them with lavender-oil.) For use 15 in china and glass decoration they are mixed with an ethereal oil, such as layender-oil. This mixture or solution is applied in a thin coat to the to-be-decorated glass or china and then burned in, leaving a thin bright firmly- 20 attached film of the metal where the ceramic luster was applied. Generally the lustrous preparations of silver, gold, and platinum are produced and employed for decorative purposes as aforesaid. The lusters of the other 25 metals of the platinum group have been little used in glass and china decoration, since they offer no decorative advantages over the platinum preparation; but they can be prepared and burned in in the same manner as the 30 platinum luster.

The lusters which I use for my incandescents are those of the highly-infusible metals of the platinum group, such as osmium, ruthenium, rhodium, and iridium.

40 I produce my incandescent as follows: With a mold or in any other convenient manner I form a luminous earth or a mixture of two or more luminous earths into the shape I desire for my incandescent, preferably a 45 hollow cylinder, Fig. 1, a curved tube, Fig. 2 or Fig. 3, or a similar form. I then heat it to redness, preferably in a muffle, by which it gains materially in hardness and consistency, if it be wanting in these respects. After 50 cooling an above-described ceramic lustrous preparation of one or more of the highly-infusible metals of the platinum group in mixture or solution with an ethereal oil is applied to the to-be-incandescent body in the form of 55 a stripe or in such other form as is best adapted to the form of the incandescent body. If the incandescent body is in the form of a tube or hollow cylinder, I coat the interior surface with the mixture or solution. I then 60 burn the ceramic lustrous preparation in by heating the to-be-incandescent body after the manner generally in use in the ceramic industry. Thus I obtain upon the said incandescent body a thin firmly-adherent strip (65 *b*, Fig. 5) or film (*b*, Fig. 4) of metal, which when the incandescent is placed in electric circuit serves in the first instance to conduct

the current, and thus heat the incandescent body *a* until it itself becomes a conductor, when the current passes through the incandescent and heats it to incandescence.

Owing to the highly-refractory character of the metal strip or film I employ for the initial heating current, it is not dissipated or destroyed by the passage of the current nor 75 does it require to be cut out of the current when my lamp is in operation. It takes care of itself.

As to the material of which my incandescent body *a* is composed, one of the oxids of 80 the earthy metals which become luminous at an elevated temperature may be used or mixtures of two or more of the same—as, for example, lime, baryta, strontia, magnesia, the oxids of thorium, cerium, zirconium, erbium, &c. 85

In molding or forming the incandescent body if the material selected is such as to render increased cohesion desirable a small quantity of phosphoric, silicic, or boric acid, or the like may be added in admixture as a 90 binding material.

Magnesia with a small quantity of thorium oxid, the latter containing about one per cent. of cerium oxid in admixture, I find to be well adapted for my incandescent body. At the 95 proper temperature it illuminates well, and, for example, a hollow cylinder, Fig. 1, may be easily made by mixing magnesia with water, adding ten to twenty per cent. of thorium oxid containing about one per cent. of cerium 100 oxid and about one per cent. of silicic acid or the like as a binder and then subjecting the mass to strong pressure in a mold. Incandescent bodies of other suitable materials may be made in the same manner.

As to the form of my incandescent, the hollow cylinder, Fig. 1, is perhaps the most convenient and useful form, since it is easy to make and has a large lighting-surface, and it is the form I prefer; but I do not restrict myself to that precise form, since it is obvious that other forms (for instance, Figs. 2, 3, or 5) will answer the purpose more or less perfectly.

If the hollow cylinder be used, the following 115 dimensions will be found generally useful, though the size of course depends largely on the amount of light desired and the strength and voltage of the electric current used: Length of cylinder, from five to fifteen millimeters; thickness of wall, one to five millimeters; internal diameter, from two to three millimeters.

In producing the preliminary conductor *b* I use for this purpose the mixture or solution 125 with an ethereal oil of a ceramic luster having as its basis osmium, iridium, rhodium, ruthenium, or a mixture of two or more of these metals and then burn said luster in, as is done in the decoration of china, glass, &c., 130 when these lusters are used for that purpose.

If the ceramic luster contains much osmium or other oxidizable metal, the operation of burning in should be conducted in a closed

muffle in the presence of a reducing or neutral gas—such as carbonic acid, hydrogen, or illuminating-gas—as is well known. If the mixture contains iridium, it is preferable to burn it in a closed muffle filled with hydrogen alone and not with illuminating-gas in order to prevent the formation of iridium carbide, (Ir.C<sub>4</sub>.) Indeed, in any case it is safer, and therefore preferable, to burn in in a closed muffle in the presence of hydrogen alone, since this method is adapted to all lustres. Of course such a ceramic luster should be chosen as will after burning in leave a metallic film of a sufficiently-high melting-point not to fuse on the passage of the electric current.

Generally a single application and firing of the luster gives sufficient thickness; but where the solution or mixture of the luster is so poor in luster as to give too thin a coating in one operation the operation of coating and firing may be repeated until a satisfactory coating has been obtained.

I have obtained my best results with a hollow cylinder of magnesia mixed with about twenty per cent. of oxid of thorium containing about one per cent. of cerium coated within with osmium; but instead of the magnesia lime, baryta, or any of the hereinbefore-mentioned earths may be used, or the coating may be of ruthenium or rhodium and good results may be obtained.

My incandescent operates as follows: When a suitable electric current is passed through the metallic coating *b* of the incandescent, which we will assume is in the form of a hollow cylinder, Fig. 1, the coating becomes heated, because of its thinness and consequent resistance to the current. This in turn heats the body *a*, which when so heated is a conductor of electricity. The entire cylinder then speedily begins to glow and emits a brilliant light.

My incandescent may be used as an illuminant in the open air provided the metallic coating consists of a highly - inoxidizable metal; but if it contains any material quantity of osmium the incandescent should be protected by a bulb that is exhausted or filled 50 with a neutral or reducing gas.

Having thus described my invention, what I claim as new, and desire to secure by Letters Patent, is—

1. The within-described method of making

incandescents adapted to incandescent electric lighting, which consists in first: forming a body of the desired shape from one or more of those oxids of the earthy metals which become conductive and luminous at elevated temperatures; second, applying to the surface of the body so formed a partial coating of a ceramic lustrous preparation of one or more of the highly - infusible metals of the platinum group; and lastly, burning said ceramic preparation in, to reduce the same to a metallic form and cover the coated portion of said body with a superficial adherent film-like deposit of such metal or metals.

2. As a new article of manufacture, an incandescent adapted to electric lighting, which consists of a body composed of one or more of those oxids of the earthy metals which become conductive and luminous at elevated temperatures, provided with an initial heating device consisting of a film-like coherent and adherent partial coating of one or more of the highly-infusible metals of the platinum group produced by burning in a ceramic luster of the same.

3. As a new article of manufacture, an incandescent adapted to electric lighting, which consists of a body composed of one or more of those oxids of the earthy metals which become conductive and luminous at elevated temperatures, provided with an initial heating device consisting of a film-like coherent and adherent partial coating of one or more of the highly-infusible metals of the platinum group, as produced for example by burning in a ceramic luster of the same.

4. As a new article of manufacture, an incandescent adapted to incandescent electric lighting, which consists of a hollow body composed of one or more of those oxids of the earthy metals which become conductive and luminous at elevated temperatures, provided with an initial heating device consisting of an interior adherent coating of one or more of the highly-infusible metals of the platinum group.

Signed at Frankfort-on-the-Main, in the Empire of Germany, this 1st day of June, A. D. 1899.

GEORG ALEFELD.

Witnesses:

JEAN GRUND,  
WILHELM HESS.